

# UNITED STATES PATENT OFFICE.

MYRTIL KAHN AND ANTON OSSENBECK, OF ELBERFELD, GERMANY, ASSIGNEES TO  
FARBENFABRIKEN VORM. FRIEDR. BAYER & CO., OF ELBERFELD, GERMANY, A  
CORPORATION OF GERMANY.

## DYE-BATH AND PROCESS OF DYEING.

1,025,273.

Specification of Letters Patent.

Patented May 7, 1912.

No Drawing.

Application filed September 7, 1911. Serial No. 648,191.

To all whom it may concern:

Be it known that we, MYRTIL KAHN and ANTON OSSENBECK, doctors of philosophy, chemists, citizens of the German Empire, 5 residing at Elberfeld, Germany, have invented new and useful Improvements in Dye-Baths and Processes of Dyeing, of which the following is a specification.

We have found that blue fast shades on 10 wool can be obtained by dyeing according to the one-bath method the azo dye: 4-chloro-2-aminophenol-6-sulfonic-acid-azo-beta-naphthol on wool in the presence of a chrome mordant.

15 In order to illustrate the new process more fully the following example is given, the parts being by weight:—Prepare the dye-bath with 4 per cent. of the dye: 4-chloro-2-aminophenol-6-sulfonic acid+beta-naphthol, bring to the boil, add 2 per cent. of potassium bichromate, enter the wool at 20 60-80° C., bring to the boil, boil during  $\frac{3}{4}$  hour and add slowly 2-3 per cent. of acetic acid and continue boiling for 1-1½ hours. 25 A deep dark blue fast shade is thus obtained. Another chrome compound or another acid can be used.

We claim:—

1. In the art of dyeing wool the improve- 20

ment consisting in dyeing wool from an acid bath containing a chrome mordant and the dye: 4-chloro-2-aminophenol-6-sulfonic-acid-azo-beta-naphthol, substantially as described. 30

2. In the art of dyeing wool the improvement consisting in dyeing wool from an acid bath containing potassium bichromate and the dye: 4-chloro-2-aminophenol-6-sulfonic-acid-azo-beta-naphthol, substantially as described. 35

3. An acid dye-bath comprising the azo-dye: 4-chloro-2-aminophenol-6-sulfonic-acid-azo-beta-naphthol and a chrome mordant, substantially as described. 40

4. An acid dye-bath comprising the azo-dye: 4-chloro-2-aminophenol-6-sulfonic-acid-azo-beta-naphthol and potassium bichromate, substantially as described. 45

In testimony whereof we have hereunto set our hands in the presence of two subscribing witnesses. 50

MYRTIL KAHN. [L. S.]  
ANTON OSSENBECK. [L. S.]

Witnesses:

L. NUFER,  
A. F. NUFER.